

# UNITED STATES PATENT OFFICE

2,306,976

## PROCESS FOR THE REMOVAL FROM CAST IRON THE OXIDES INTRODUCED THERE- IN AND OTHER FOREIGN INCLUSIONS

Nicholas L. Pedersen, Clifton, N. J.

No Drawing. Application March 23, 1942,  
Serial No. 435,832

1 Claim. (Cl. 75—53)

This invention relates to the process of removing the oxides and other foreign inclusions introduced into cast iron in its various forms known as gray iron, semi-steel and alloyed cast iron in one single treatment by means of adding a distinct chemical known as sodium silico fluoride to the molten metal as a ladle scavenger or flux, or added to the stream of hot iron in the spout as it leaves the cupola and has for its object the purpose of furnishing to the trade a superior casting product at a price at par with that charged for the product now cast from the untreated metal.

I have found that sodium silico fluoride when added to the molten iron in amounts up to five pounds for every 2000 pounds of iron to be treated will result in a cast iron more free of blow

holes and sponge, cleaner, closer grained, stronger and tougher than cast iron which has not been treated by this chemical. The machinability of the casting is not impaired thereby.

5 Due to the simplicity of the treatment and the small cost involved, which is offset by the reduction in rejects due to such defects as blow holes, sponge and slag, the casting product can be manufactured and sold at a price at par with 10 castings made from the ordinary run of untreated metal.

I claim:

The process of removing from cast iron the oxides introduced therein and other foreign inclusions by adding sodium silico fluoride to the molten cast iron.

NICHOLAS L. PEDERSEN.